

June 4, 1940.

T. L. OSBORNE ET AL

2,203,232

MEANS FOR PROTECTING SHEATHS OF ELECTRIC CABLES, PIPES,  
AND OTHER METAL ARTICLES AGAINST CORROSION

Filed May 11, 1938

Fig. 1.



Fig. 2.



INVENTORS  
THOMAS LLOYD OSBORNE  
and HAROLD JOHN ALLCOCK

BY  
Scribner, Keeler & Poncela

ATTORNEYS

## UNITED STATES PATENT OFFICE

2,203,232

MEANS FOR PROTECTING SHEATHS OF  
ELECTRIC CABLES, PIPES, AND OTHER  
METAL ARTICLES AGAINST CORROSIONThomas Lloyd Osborne and Harold John Allcock,  
Belvedere, Kent, England, assignors to Cal-  
lender's Cable and Construction Company  
Limited, London, England, a British companyApplication May 11, 1938, Serial No. 207,301  
In Great Britain May 27, 1937

## 4 Claims. (CL. 91—68)

This invention is concerned with the production of wrappings, of impregnated paper and cotton and other textile fabrics formed of natural cellulosic materials, such as are used for protecting sheaths of electric cables, pipes and other metal articles against corrosion and proceeds from the discovery that when natural cellulosic material is subjected to a vacuum and heat in the presence of rosin it undergoes a chemical change on the surface which appears to be an esterification, cellulose rosinate being produced. This reaction, which is accompanied by the production of water that must be removed for the reaction to continue, can be employed, as described and claimed in the specification of co-pending United States application, Serial No. 207,299 filed on May 11, 1938, for the purpose of making paper or fabric resistant to water.

In accordance with the present invention we provide a cable sheath, pipe or other metal body with a protective covering comprising one or more wrappings of a material, consisting of paper or cotton or other fabric formed from natural cellulosic material, of which the fibres have been coated with a film of cellulose rosinate by drying the material by subjecting it to heat and a vacuum in the presence of rosin and of which the passages between the coated fibres have been sealed by impregnating the vacuum dried material with a water excluding compound. The coating of cellulose rosinate on the fibres reduces the water absorptive capacity of the material and to a large extent overcomes the difficulty experienced with existing coverings formed of paper or fabric impregnated with a water excluding compound which merely fills the passages between the fibres, of preventing the passage of moisture through the fabric by way of the fibres themselves. In the case of paper and felted fabric, the cellulose rosinate coating also has the advantage of giving it the power to resist the softening and disintegrating action of water.

The accompanying drawing shows by way of example a length of a lead sheathed electric cable furnished with a corrosion resistant protective covering constructed in accordance with the invention. In the drawing

Figure 1 is a perspective view of the protected cable from which portions of the component parts have been removed to expose the construction thereof, and

Figure 2 is a cross-sectional view, on an enlarged scale, of the cable shown in Figure 1.

The illustrated cable comprises a stranded

conductor 1 surrounded by a body of dielectric 2 and a seamless lead or lead alloy sheath 3. Surrounding the sheath 3 are two wrappings 4 and 5 of cellulosic material, for instance, paper or cotton tape, of which the fibres are coated 5 with a film of cellulose rosinate and of which the interstices between the coated fibres are sealed by a water excluding compound. The wrappings 4 and 5 are so arranged that the small gap between successive turns of the wrapping 4 are bridged by the turns of the wrapping 5. Over the wrapping 5 is a wrapping of fabric material 6, for instance, hessian, on which is arranged a single layer of wire armouring 7 in the usual manner.

The rosin required for the formation of the water resistant film on the fibres of the material used in the construction of the improved protective covering may in general be applied in any way which brings it into intimate contact 23 with the fibres of the paper or fabric. This is, of course, subject to the qualification that the method does not involve the use of any material which disadvantageously affects the paper or fabric, either in its structure or in its properties required for its subsequent use. The rosin may, for instance, be applied in solution or in the form of a suspension. A solution may, for instance, be made by the aid of trichlorethylene, alcohol or other organic solvent for rosin. 38 Satisfactory results are obtained if the solution strength is such as to leave about 5 parts by weight of rosin in 100 parts by weight of paper or fabric. The paper or fabric is soaked in the solution or suspension, for instance, by running 38 it through a bath of the solution or suspension, and the solvent or suspension medium may be removed by drying in air or under a pressure less than atmospheric pressure. In the case of paper the rosin may be incorporated in the process of manufacturing the paper, for instance, during the beating stage. Conveniently a rosin-sized paper containing about 5% by weight of rosin may be employed.

The rosin-containing material thus produced 45 or obtained is treated in accordance with the invention by heat drying it under vacuum until the reaction has been completed or substantially completed. A suitable treatment comprises drying rosin-containing material for a period varying from about 20 to about 50 hours at a temperature of about 120° C. at an absolute pressure which at the end of the process is not greater than 1 mm. of mercury. This treatment also has the advantage that it leaves the paper or fabric 55

dry and with little tendency to take up moisture. The treatment can therefore be applied to the paper or fabric while in rolls and need not immediately precede the process of impregnating with water excluding compound. The flexibility of the material is not affected by the treatment.

The sealing of the passages between the coated fibres is effected by impregnating the vacuum dried material with a water excluding compound in the usual way. As examples of water excluding compounds are mentioned pitch, tar, bitumen and oil compounds. These materials penetrate into the paper or fabric and adhere to the surface thereof.

The improved protective covering has greatly improved resistance to the penetration of moisture and to the softening effect of any moisture which does penetrate into it. An indication of this is provided by comparing the tensile strength of ordinary paper impregnated with bitumen and then saturated with water with a similar grade of paper vacuum dried in the presence of rosin in accordance with the invention and subsequently impregnated with bitumen and then saturated with water. The following figures have been obtained for a particular grade of paper.

|    | Sample                                                                              | Breaking load after soaking in water at 60° C. for 24 hours |
|----|-------------------------------------------------------------------------------------|-------------------------------------------------------------|
|    |                                                                                     | Pounds                                                      |
| 30 | Ordinary paper impregnated with bitumen                                             | 6.25                                                        |
| 35 | Paper vacuum dried in the presence of rosin and afterwards impregnated with bitumen | 10.0                                                        |

What we claim as our invention is:

1. A corrosion-resistant protective covering for electric cable sheaths, pipes, rods and like arti-

cles, comprising at least one wrapping of a material, formed from natural fibrous cellulosic substance, of which the fibres are coated with a water-resistant film of cellulose rosinate formed in situ and of which the passages between the coated fibres are sealed by a water-excluding compound.

2. A corrosion-resistant protective covering for electric cable sheaths, pipes, rods and like articles, comprising at least one wrapping of a material, formed from natural fibrous cellulosic substance, of which the fibres are individually coated with a water-resistant film consisting of the reaction product of the surface cellulose of the fibers and rosin and of which the passages between the coated fibres are sealed by a water-excluding compound.

3. A corrosion-resistant protective covering for electric cable sheaths, pipes, rods and like articles, comprising at least one wrapping of a material, formed from natural fibrous cellulosic substance, of which the fibres are individually coated with a water-resistant film consisting of the reaction product of the surface cellulose of the fibres and rosin and of which the passages between the coated fibres are sealed by bituminous compound.

4. A corrosion-resisting protective covering for electric cable sheaths, pipes, rods, and like articles, comprising at least one wrapping of a material formed from natural fibrous cellulosic substances, of which the fibres have been superficially esterified by treatment with rosin, and of which the passages between the superficially esterified fibres are sealed by a water-excluding compound.

THOMAS LLOYD OSBORNE.  
HAROLD JOHN ALLCOCK.